

# United States Patent [19]

Kay et al.

[11] 3,750,275

[45] Aug. 7, 1973

[54] **MANUFACTURE OF ELECTRICAL COILS**

[75] Inventors: **Albert Ernest Kay; Arthur Wellesley Stewart Clark**, both of London, England

[73] Assignee: **Aluminium Foils Limited**, London, England

[22] Filed: **Aug. 23, 1971**

[21] Appl. No.: **174,203**

[30] **Foreign Application Priority Data**

Aug. 28, 1970 Great Britain ..... 41,513/70

[52] U.S. Cl. .... **29/605, 29/25.42, 336/205, 336/206**

[51] Int. Cl. .... **H01f 7/06**

[58] Field of Search ..... **29/605, 25.42; 336/205, 206**

[56] **References Cited**

UNITED STATES PATENTS

3,518,755 7/1970 Olson ..... 29/605  
3,545,078 12/1970 Lightner ..... 29/605

*Primary Examiner*—Charles W. Lanham

*Assistant Examiner*—Carl E. Hall

*Attorney*—Holcombe, Wetherill & Brisebois

[57] **ABSTRACT**

A lacquer insulated metal foil coil has continuous interturn and end face insulation the latter being produced from lacquer exuded from between the turns in a heating step.

**2 Claims, No Drawings**

## MANUFACTURE OF ELECTRICAL COILS

This invention is concerned with improvements in and relating to the manufacture of electrical coils from metal foil, which coils are suitable for electro-magnets, solenoids or other inductors. In particular it concerns the production of coils consisting of ribbons of foil coated with an adherent insulating lacquer.

The method of production of such coils by slitting a wide web of aluminium foil into ribbons of suitable width is well known. A normal method of providing the interturn insulation is by interleaving the ribbon with a ribbon of paper or other non-conducting film during the operation of winding the coil. It is well known that the ribbon of non-conductor should be a little wider than the metal foil and should be positioned so that there is an overhang on both edges. By this precaution it is possible to avoid the danger of short circuits between adjacent turns due to deformation of the edges of the metal strip. When use is made of an adherent insulating lacquer to separate the turns, overhanging edges cannot be obtained from the slitting machine. Additional operations, known as edge conditioning, have to be performed to eliminate edge deformation or rags and to provide a longer path between the conductors than the interturn gap due to the thickness of the lacquer. This effect can be provided by a process of etching in which a liquid is used which will dissolve the metal without affecting the lacquer. Such etching processes have been described for the manufacture of capacitors and solenoids. The etching processes suffer from the drawback, besides being an additional manufacturing operation, that they are wet processes and require thorough washing followed by drying to ensure the complete removal of strong reagents used in the etch and all water which might tend to set up corrosion of the metal conductor within the coil. In addition, very careful control of the metal removal process is required to ensure that it is uniform and that the etchant does not penetrate between the metal and the lacquer, which undercutting weakens the overhanging lacquer. There is a further difficulty that the width of the conductor, and therefore its cross sectional area, is dependent for its accuracy on the control of the etch, which is much less accurate in establishing the width of the ribbon than the slitting machine.

The present invention provides a process for the manufacture of an electrical coil including the steps of coating a metal foil with an adherent insulating lacquer, slitting the coated foil and winding to a coil, in which process there is used as insulating lacquer a lacquer composition of a thermosetting nature and capable of undergoing by the action of heat a curing or further curing whereby the lacquer is first rendered fluid and finally sets, the tension applied in winding the coil is sufficient to cause or allow the fluid lacquer to exude from between the turns of the coil, and the wound coil is subjected to such a degree of temperature and for such a time that exudation and setting produce a final coil in which the interturn insulating effect is preserved and in addition an edge insulation is provided. When the coil is of other than circular shape, the winding tension may not give a uniform interturn pressure at all parts of the coil and this pressure may have to be augmented by the use of a jig with correctly positioned pressure plates during the curing phase.

By this process the above difficulties can be overcome. The lacquer can be applied by any of the estab-

lished methods of coating and the ribbons of coated foil can be slit to the desired width by any well known slitting machine taking the usual care to produce an edge as free from deformation as possible and with the edge of the lacquer layer laying flush with the edge of the metal conductor. It is however necessary to control the tension applied to the conductor as it is being wound within the limits described.

For this purpose it is not necessary to depart from the ordinary process of winding using, for example, the Kampf reeling machine normally employed in the aluminium foil converting industry. All that is required is that in such a winding operation the tension be carefully maintained throughout. The control of the wander of the turns, i.e., the variation in the relative positions of the superposed edges, should also be carefully observed. Where, in spite of such control, the degree of uniformity at the edge of the coil is insufficient to produce a satisfactory result from the use of the process of the invention, it may be necessary to face up the edge in some conventional manner of a mechanical or chemical nature.

When the coil has been wound to the desired size, and terminations attached as required, it is heated in an oven. Under the influence of the heat, the lacquer or a part of it liquefies and expands, or merely liquefies, and the pressure produced as a result of the tension of winding the coil, or by the expansion of the lacquer, causes the lacquer, or part of it, to flow and to be exuded beyond the edge of the conductor. Furthermore, the lacquer being of a thermosetting nature, by the continued action of the heat it reacts and becomes rigid. When the coil is removed from the oven and allowed to cool, it has become a solid mass held together by the adhesive nature of the thermoset lacquer which forms the insulating layer between the turns. Moreover the faces of the coil are now usually covered by a continuous film formed by that part of the lacquer which was exuded. By this means the conducting turns are separated from each other and protected from outside influences.

It will be understood that no intermediate process between slitting the foil into ribbons and winding the desired coil is required, excepting only in the circumstances described above where it is necessary to correct deficiencies in the winding technique. Further the width of the metal conductor remains as produced by the setting of the slitting knives or as resulting from the facing operation.

In a modification of the process of the invention, instead of the lacquer composition being of a thermosetting nature it is of a thermoplastic nature, the tension applied in winding the coil is sufficient to cause or allow the fluid lacquer to exude from between the turns of the coil, and the wound coil is subjected to such a degree of temperature and for such a time that by exudation, then followed by cooling, a final coil is produced in which the interturn insulating effect is preserved and in addition an edge insulation is provided.

In this case the resulting coil is of more limited applicability since it can only be used at temperatures so far below the melting point of the thermoplastic resin that no movement within the coil takes place in service.

The practice of this invention obviously requires that the original lacquer film be produced in a dry and non-tacky condition and that, in the case of a thermosetting lacquer, it can later be irreversibly reacted by heat on

one occasion. Within certain limits, to allow for exudation, the quantity of lacquer applied is in inverse proportion to the width of the ribbon used to form the coil, the less the width of the ribbon the greater the thickness of the lacquer required. For ribbons of more than a certain width, however, this proportionality is no longer important. The quantity of lacquer required is in direct proportion to the thickness of the ribbon and is also markedly affected by the precision of the alignment of the convolutions one upon the other. Furthermore the tension applied to the ribbon by the coil winding machine must be sufficient to produce a minimum interturn pressure without which the lacquer will not be exuded. Lastly, also in the case of a thermosetting lacquer the temperature must be above a certain minimum to ensure that the time available for flow to take place is suitably related to the gel time of the lacquer.

The type of lacquers which may be used in this invention is very varied. Obviously the dry lacquer solids must form a layer which is attached to the metal sufficiently strongly to be wound, unwound and slit without damage at a convenient temperature. At a higher temperature the resin solids must melt to a liquid whose viscosity is sufficient to allow it to flow under the pressure applied to it. It is also useful if the lacquer is of such a type that it can form two phases on melting. One of the phases, being more mobile than the other, exudes more rapidly leaving the other to maintain the separation between the adjacent convolutions. One component of the lacquer may be solid from the class of finely ground thermally inert non-conducting materials. Such a solid material remaining between the convolutions maintains the integrity of the insulation between them. In the case of a thermosetting lacquer, at a still higher temperature, reaction must commence within the molten lacquer solids leading to a rise in viscosity and gelation consequent upon cross-linking. The range between these two temperatures may be termed the critical temperature range. There is thus a relationship between the viscosity and the applied pressure over the critical temperature range. The amount by which the lacquer will move will also depend on the length of time that it remains within the critical temperature range. The period can be lengthened if required by reducing the degree of heating of the coil but cannot be reduced below the minimum time required by the coil to absorb heat. Since cross-linking may not occur instantaneously on reaching the cure initiation temperature, the time within the critical temperature range may be varied by choosing different properties of curing agent or by choosing more or less reactive curing agents.

It follows from the above that in the practice of this invention, it is possible to fit the mechanics, i.e., the winding tension, the coating weight and the width, to the lacquer available or to accept given values of these and to select a lacquer to suit, or both approaches may be partially adopted.

Lacquer systems which are useful include solid epichlorhydrin resins blended with solid curing agents, e.g., dicyandiamide, phenol, cresol or similar aromatic hydroxylated molecules after resinification with formaldehyde, or similar well known urea-formaldehyde or melamine-formaldehyde resins: solid polyhydroxy alcohols which react with isocyanates blocked so that they remain inactive below a certain temperature may also be used. Other well known lacquer systems are also

suitable. Application is usually from solvent solution but other methods e.g., hot melt, electrostatic deposition or powder coating may be used provided they meet the requirements given above.

5 The following Examples illustrate the invention; (R) means Registered Trade Mark:

#### EXAMPLE 1

The winding of a solenoid coil is constructed from 10 fully annealed commercial purity (99.2 percent) aluminium foil which has been reduced by rolling to a nominal thickness of 0.015 mm. A web of this material, approximately 720 mm wide, is coated with a solution of:

15 Epoxy Resin — Shell "Epikote" (R) 1001 37 parts by weight

Phenolic Resin — "Bakelite" (R) R 18973 11 parts by weight

20 in Methyl Ethyl ketone (m.e.k.) + methylated spirit in the ratio 2:1 52 parts by weight.

Before application, the viscosity of this solution was adjusted with additional solvent so that a dry weight of 4.3 grams/sq. metre remained on the foil surface after evaporation of the solvent. The coating and drying were carried out on a roller application coating machine with a steam heated drying drum whose temperature did not exceed 140°C. The coated web was reeled up and conveyed to store in readiness for the next operation. Tests on this foil showed that the temperature at which the coating began to adhere to plain foil was 63°C. There was no danger in keeping the reel in store at normal room temperature. When heated to 190°C for one hour the coating lost all solubility in m.e.k. and could not be removed from the foil by pulling with Scotch Tape. A lap joint made between the coated foil and plain foil at 190°C with a pressure of 0.04 kg/sq. cm withstood a sheer load of 200 g. on a 4 sq.cm area at a temperature of 190°C. This web of coated foil was

30 35 40 45 50 55 60

slit and wound into a set of 26 mm wide reels on 1mm internal diameter cores until a final diameter of 108 mm was reached. This was done on a Kampf reeling machine as is usual in the aluminium foil converting industry. Care was taken to maintain the tension in the web. After attaching a termination and securing the end, the reels were placed in an oven heated to 200°C for one hour while supported on a bar with their axes horizontal. When removed and cooled, the end faces of the reels were seen to be coated with the hardened exudate from the lacquer. Some of the coils were sectioned and it was found that the resin coating between the convolutions was 3 to 4 micrometres thick and the minimum thickness of exudate over the most protruding convolution was 6 micrometres. The electrical resistance of the coils was 17.07 ohms. This was very similar to the value of 17.86 ohms. obtained by rewinding one of the reels from the set described and interleaving it with insulating paper which overhung 2 mm. on either side of the foil conductor as described in the prior art. The coils were suitable for installation without further treatment.

#### EXAMPLE 2

In another application a solenoid coil was made for an automobile switch. The winding is made from commercial purity aluminium as before but of nominal thickness 0.018 mm. A web of this material, approxi-

mately 180 mm wide, is coated with the solvent solution of the following resinous materials:

Epoxy resin — Shell "Epikote" 1001 37 parts by weight

Heat hardening phenolic resin — "Bakelite" R 18973 5.5 parts by weight

Non-heat hardening phenolic resin "Bakelite" R 5468/1 5.5 parts by weight

This was dissolved in the solvent mixture described in Example 1 so that a dry weight of 3.66 gram/sq. metre remained on the foil surface after evaporation of the solvent. The coating and drying were carried out on a gravure roller application machine with an electrically heated drying plate whose temperature did not exceed 140°C. The coated reel was then stored until required for the next operation. Tests carried out as in Example 1 showed similar performance. The web of coated foil was now slit into reels 26 mm wide on 58 mm diameter cores which were transferred to a coil winding machine. The ribbon of coated foil was then wound onto a brass core of 18 mm diameter until the winding diameter became 34 mm. This required 27.42 m of coated foil. Care was taken to maintain tension in the web and to control the wander. A termination was attached to the end of the winding and the end secured by suitable adhesive tape. After treatment in an oven at 200°C for one hour supported by a bar with its axis horizontal, the coil was allowed to cool. The end faces were found to be completely covered with the hardened exudate. The resistance of the winding, measured between the termination and the brass core which is in contact with the uncoated side of the first convolution wound, was found to be 1.603 ohm, being about 95 percent of the theoretical 1.681 ohms calculated from the length, width and nominal thickness of the aluminium. When the coil was sectioned it was found that the average thickness of insulation between convolutions was 3  $\mu$ m. The winding showed a degree of wandering giving a mean step height (i.e., the protuberance of the edge of any coil turn beyond the innermost coil turn edge) of 60  $\mu$ m. The edge of the convolutions were completely covered by a resinous layer 100 to 150  $\mu$ m thick with a minimum of 40  $\mu$ m over the most protruding convolutions.

### EXAMPLE 3

A solenoid coil is concerned whose ampere-turns figure was required to be 1935 on a 12 volt supply. Calculation showed that 333 turns of ribbon conductor 26 mm wide by 0.015 mm thick was required. A ribbon coated foil prepared in a manner similar to that described in Example 2 was taken to a coil winding machine and the required number of turns wound on to a 22.5 mm o.d. 2.75 mm wall thickness core using great care to maintain tension in the strip and to control the wander of the ribbon during winding. A termination was attached to the end of the conductor ribbon and the end secured with suitable adhesive tape. A jig was made which consisted of two parallel strips of polytetrafluoroethylene attached to a base so that they were held vertically with their long edge horizontal and separated by 22.5 mm equal to the o.d. of the winding core used. The upper edges of the strips had previously been chamfered off at 45° so that a knife edge existed on the inner edges of the strips. A number of coils prepared as described above were laid on this jig with their axes vertical and the cores centralised between the two

PTFE strips. The coils did not touch each other. In one experimental run a block was inserted to carry the weight of the core and in another this was omitted. The jig carrying the coils was placed in an oven at 200°C for 1 hour. When removed and cooled the coils were found to be covered on both faces with the hardened exudate. The resistances of the coils were typically 2.05 or 2.04 ohms well within the tolerance allowed and the coils were . . . suitable for their designed duty. On sectioning 10 sample coils the thickness of insulation was found to be approximately 3  $\mu$ m. The mean step height was 33  $\mu$ m and the average thickness of the exudate was 70  $\mu$ m with a minimum of 5  $\mu$ m over the most protuberant convolution.

### EXAMPLE 4

It will have been revealed in the previous Examples that it is preferred that the thickness of the metal ribbon and the thickness of the initial coating should be in the approximate ratio of 4 to 1 or less. This assures an adequate supply of exuded lacquer to cover the edge faces of the coils. In one case it was necessary to use a ribbon of foil 0.096 mm thick carrying a fully thermoset insulating lacquer coating on one side. For the purpose of this invention it would have been preferred to apply approximately 25 g/sq.m of the coating described in Example 1 to the other side of the foil ribbon. The limitations of the coating machinery available were such that it was not possible to apply more than 6.75 g/sq.m. of the coating. Since this was less than was desired, the following procedure was adopted to make the best use of the quantity available, by reducing the turn to turn misalignment to the minimum. The coated web was slit to 27 mm width and this ribbon taken to the coil winding machine and wound into a coil on 30 mm diameter core taking care to maintain tension and to control the wander to within  $\pm 0.5$  mm. The end of the winding was secured with suitable insulating tape and the coil mounted in a lathe. It was then machined so that both faces were smooth and 26 mm apart. The faces were then brushed with a stiff brush to remove as many rags as possible and then washed over with Tuckers Etch which remained in contact with the surface for about 30 seconds before being washed off. Since the contact time had been so short there was no penetration into the coil and drying was simple. Examination of the surface showed that the convolutions were clear of each other. The coil was then placed in an oven at 200°C for one hour supported with its axis horizontal on a bar through the core. When removed and cooled, the edge faces were found to be protected by a thin film of exudate. On sectioning this was found to cover the edges of the convolutions to a depth of about 5 micrometres. In this coil the interturn insulation was provided by the thermoset insulating lacquer mentioned above. It may appear that the advantage of the invention is lost by the need to use an etch but this is not so since the amount of etching and the time spent doing it are much reduced compared with the prior art. Rather is this regarded as a method whereby the process of this invention can be extended to be useful when the coating thickness is limited and the foil or strip is thick.

### EXAMPLE 5

The method of preparation described in the foregoing examples can also be applied when the lacquer used

does not possess thermosetting properties. A ribbon of foil 0.10 mm nominal thickness and 30 mm wide, was coated with a tough polyamide resin, "Versalon" (R) 1175, supplied by Cray Valley Products Ltd.. This is a thermoplastic material with a Ball & Ring softening point of 170°-180°C. The material which is supplied in granular form was dissolved at 100 g/l in a mixture of toluene and ethyl alcohol as recommended by the makers. This solution was coated onto the ribbon of foil using a wire-wound spreader bar and the solvent evaporated to leave a dry coating weight of 12.0 g/sq.m.. After cooling, the ribbon of foil was reeled up ready for the next process which was to wind a coil on a 30 mm diameter core. Winding tension was applied so that the aluminium was elastically stretched and a firm dense winding produced, and the end firmly secured to retain this tension. The coil was then mounted in a lathe and machined so that both faces were smooth and 26 mm apart. The faces were then brushed to remove as many rags as possible and then washed over with Tuckers Etch. The faces were then rinsed and dried. Examination of the surfaces showed that the convolutions were clear of each other. The coil was then heated in an oven until it reached a temperature of 246°C being supported on polytetrafluoroethylene knife edges as previously described. The coil was then allowed to cool without disturbance. When it was cold it was seen that

the surfaces were covered with a thin film of exuded "Versalon" 1175. The coil was suitable for use on duties which did not cause its temperature to rise above ambient.

5 We claim:

1. A process for the manufacture of an electrical coil, comprising the steps of

- 10 1. preparing a web of metal foil coated with a solid dry coating of a lacquer that is initially heat-melted and finally heat-curable to form a thermoset lacquer;
- 15 2. longitudinally slitting said foil having said dry coating to produce a ribbon having cut longitudinal edges, said coating extending to said edges;
- 20 3. uniformly winding said ribbon under tension to form a coil with closely superposed edges;
- 25 4. attaching electrical terminations to said coil; and
5. subjecting said coil to controlled heat; whereby sufficient of said lacquer is exuded from between said turns on melting to produce continuous end face insulation for the coil while leaving adequate lacquer for inter-turn insulation, said heating being continued to cure said lacquer.

2. A process as claimed in claim 1, in which the end faces of the wound coil containing uncured lacquer are subjected to a facing-up step prior to the curing step.

\* \* \* \* \*

30

35

40

45

50

55

60

65